

C. H. SCHROERS.

CARBON ELECTRODE HAVING PROTECTIVE COVERING, AND PROCESS FOR PRODUCING SAME.  
APPLICATION FILED MAR. 14, 1913.

1,088,734.

Patented Mar. 3, 1914.

Fig. 1.



Fig. 2.



Witnesses:-

Charles B. Crompton.

John A. Percival.

C. H. Schroers.  
Inventor

By S. Broya and Marks  
Attorney.

# UNITED STATES PATENT OFFICE.

CARL HERMANN SCHROERS, OF DUISBURG-MEIDERICH, GERMANY, ASSIGNOR TO  
GESELLSCHAFT FÜR TEERVERWERTUNG M. B. H., OF DUISBURG-MEIDERICH,  
GERMANY.

## CARBON ELECTRODE HAVING PROTECTIVE COVERING, AND PROCESS FOR PRODUCING SAME.

1,088,734.

Specification of Letters Patent.

Patented Mar. 3, 1914.

Application filed March 14, 1913. Serial No. 754,344.

To all whom it may concern:

Be it known that I, CARL HERMANN SCHROERS, a subject of the German Emperor, residing at No. 57 Neumühlerstrasse, 5 Duisburg-Meiderich, Germany, have invented certain new and useful Improvements in Carbon Electrodes Having Protective Covering, and Processes for Producing Same, of which the following is a specification.

10 It is a well known fact that the carbon electrodes in electric furnaces are subject to considerable wasting by burning away under the action of air or other oxidizing gases between the sockets or terminals of 15 the furnace electrodes and the melting hearth. If the electrode is left unprotected thus burning away of the portion exposed to the gases is liable to render the electrode prematurely useless. It has already been 20 proposed to remove this drawback by covering the surface of the electrode at the endangered places with wire fabric, fire proof materials and sheet metal casings for the purpose of increasing the life of the carbon blocks. With the same object it has also 25 been proposed to protect the surface of the electrodes with an electro-deposited metal covering or to render the said surface unaffected by oxidizing gases by covering the 30 same with a coating of enamel or with a glaze or vitreous layer. It has also been proposed to convert the surface of the electrode into carbids or into graphite. All 35 those proposed methods of protecting the electrodes increase the cost of the electrodes considerably because the electrodes have first to be manufactured in the usual manner and have then to be provided by a second process with the covering intended for protection against oxidizing gases.

The present invention has now for its object to provide an improved process for the production of protective coverings on carbon electrodes, more particularly for use in 45 electric furnaces.

According to this invention an efficient and yet cheap protection of the surface of the electrode is effected by pressing, rolling, hammering or otherwise embedding into the 50 surface of the electrode before the same is burned, a coating of granular materials which are unaffected by oxidizing gases, especially at high temperature. The parti-

cles of the granular materials must be arranged as closely as possible to one another. 55 The electrodes may be forced out of a receiver through a nozzle or mouthpiece or they may be rammed or pressed in a mold and in the latter case they may be subjected to a subsequent pressing operation. The selection of the granular material to be employed will depend upon whether the electrodes are to have a surface having good electrical conductivity over its entire extent or whether the electrodes are to have good 60 conducting contact surfaces only for the head and end sockets or terminals in which latter case the remaining parts of the surface of the electrodes may be protected by a bad electrical conductor against the action 65 of the oxidizing gases. In the former case there may be used for instance metals such as iron, aluminium and copper. In the latter case there may be used for instance quartz, slate, magnesite, carborundum, blast 70 furnace slag, aluminium oxid, and in fact any non-conducting materials provided that it is unaffected by oxidizing gases especially 75 at high temperature. It is immaterial for the purposes of this invention whether in the burning of the electrodes the granular material selected forms other compounds so long as these compounds retain the desired 80 granular texture and possess the above mentioned properties.

85 In selecting the protective materials to be employed, the manner of working of the furnace and the products resulting therefrom must be taken into consideration in order that materials which are injurious to the operation of the furnace may be avoided, and only materials may be chosen which are neutral or which will promote the operation 90 of the furnace.

In order that the construction of the electrode may be clearly understood reference may be had to the accompanying drawings, in which:

Figure 1 represents an elevation of an electrode provided with a resisting surface. 100 Fig. 2 shows a cross section of the electrode having a core *a* and a coating of resisting material.

What I claim is:

1. A process for the production of protective coverings on carbon electrodes, more

particularly for use in electric furnaces, which consists in providing the surfaces of the electrodes before they are burned, with a coating of closely arranged particles of granular material which is unaffected by oxidizing gases especially at high temperatures.

2. A process for the production of protective coverings on carbon electrodes, more particularly for use in electric furnaces, which consists in providing the surfaces of the electrodes before they are burned, with a coating of closely arranged particles of granular material unaffected by oxidizing gases especially at high temperatures, by

pressing, rolling, hammering, or otherwise embedding said granular material into the surfaces of the electrodes.

3. As a new article of manufacture, a carbon electrode having a protective layer of 20 closely arranged particles of granular material unaffected by oxidizing gases, embedded in its surface.

In testimony whereof I affix my signature in presence of two witnesses.

CARL HERMANN SCHROERS. [L. s.]

Witnesses:

ALBERT NUFER,  
HELEN NUFER.